# EUROPEAN PATENT SPECIFICATION

(11) **EP 0 603 941 B1**
(45) Date of publication and mention of the grant of the patent: **02.04.1997**
(21) Application number: 93203506.6
(22) Date of filing: 14.12.1993
(51) Int. Cl.: H01J 29/89

(54) **Display device comprising a display screen provided with a filtering layer**
Anzeigevorrichtung mit einem Bildschirm ausgerüstet mit einer Filterschicht
Dispositif d'affichage avec un écran de visualisation équipé d'un couche filtrante

(30) Priority: 21.12.1992 EP 92204041
(43) Date of publication of application: 29.06.1994
(73) Proprietor: Philips Electronics N.V., 5621 BA Eindhoven (NL)
(72) Inventor: Oomen, Emmanuel Wilhelmus Johannes Leonardus, NL-5656 AA Eindhoven (NL); van Lierop, Joseph Gijsbertus, NL-5656 AA Eindhoven (NL)
(74) Representative: Stolk, Steven Adolph

(56) References cited:
- EP-A- 0 335 680
- EP-A- 0 517 611
- FR-A- 2 662 022
- DATABASE WPI Week 8806, Derwent Publications Ltd., London, GB; AN 88-039121 & JP-A-62 297 142 (OIKE KOGYO) 24 December 1987

## Description

The invention relates to a display device comprising a display screen which is provided with a filtering layer comprising silicon dioxide, a black dye, and a metal oxide.

The invention also relates to a method of manufacturing a filtering layer of silicon dioxide on a display screen of a display device.

Filtering layers serving to reduce the light transmission are used on the faceplates of display devices, such as cathode ray tubes (CRTs) and liquid crystal display devices (LCD and LC-TV), to improve the contrast of the reproduced image. By virtue thereof, there is no necessity to change the glass composition of the display screen and the possibilities of bringing the light transmission to a desired value in a simple manner are increased. Such filtering layers reduce the transmission of both incident ambient light and light originating from CRT phosphors. As the filtering layers can be provided in a uniform manner, the transmission of the filtering layers is also uniform. The incident ambient light passes through the filtering layer and the glass display screen, after which it reflects off the rough phosphor layer on the inside of the display screen and again passes through the display screen and the filtering layer. If the transmissivity of the filtering layer is designated as T, the intensity of the reflected ambient light is reduced by a factor of T². Light originating from CRT phosphors passes through the filtering layer only once, so that the intensity of this light is reduced by only a factor of T, resulting in an increase of the contrast by a factor of T.

In United States Patent Specification US 4,987,338 a description is given of a cathode ray tube having a display screen provided with a filtering layer consisting of silicon dioxide and a dye having a selective light absorption which is maximal in the wavelength range of 575±20 nm. Said Patent Specification also describes a method of manufacturing such a layer. In said method an alcoholic solution of an alkoxysilane compound, such as tetraethyl orthosilicate Si(OC₂H₅)₄ (TEOS), acidified with hydrochloric acid and to which a dye is added, is spin coated onto a display screen. In this case, for example Rhodamine B is used as the dye. Silicon dioxide starts forming in said solution. By a treatment at an increased temperature, the formation of silicon dioxide is completed and a layer of silicon dioxide which also contains the dye is formed.

A disadvantage of the known filtering layer is its purplish-violet appearance which in the case of much ambient light leads to an undesired purplish background of the reproduced image. A further disadvantage of the known dyes used is that they are not resistant to light, so that when the layer is exposed to ambient light the transmission of the layer increases with passage of time, and hence the contrast-increasing effect decreases.

European patent application EP-A-517.611 discloses a cathode ray tube having a screen provided with a nonglare film comprising silica, a black dye and a metal oxide such as tin oxide or indium oxide as a conductive agent in order to produce an antistatic effect.

It is an object of the invention to provide, *inter alia,* a display device having a display screen which is provided with a filtering layer which has a non-coloured appearance, which is resistant to prolonged exposure to ambient light and to customary cleaning liquids such as ethanol and ammonium hydroxide and which additionally has the desired scratch resistance. The invention also aims at providing a simple method of manufacturing such a filtering layer on a display screen, which filtering layer may have, if desired, a high-gloss appearance.

This object is achieved by a display device as described in the opening paragraph, which is characterized according to the invention in that the metal of the oxide is selected from the group formed by Ge, Zr, Al and Ti. By incorporating a black dye in the oxidic filtering layer, the display screen obtains a neutral appearance which varies from light grey to black, depending on the concentration of said black dye. Many known black dyes are unsuitable because they are insoluble in the alcoholic solution of the alkoxysilane compounds used. Other so-called black dyes exhibit a blue or brown colour, instead of a black colour, in the filtering layer. Black dyes which are suitable for use in accordance with the invention are Orasol Black CN™ (Colour Index: Solvent Black 28) and Orasol Black RL™ (Colour Index: Solvent Black 29) available from Ciba Geigy; Zapon Black X51™ (Colour Index: Solvent Black 27) available from BASF and Lampronol Black" (Colour Index: Solvent Black 35) available from ICI. Said dyes enable high-gloss black filtering layers to be manufactured. A very suitable dye is Orasol Black CN™ (Colour Index: Solvent Black 28) because it has a high resistance to light. The chemical structural formula of the latter dye is unknown; according to the information provided by the supplier it is a mono-azo chromium complex. Dependent upon the desired transmission, the filtering layer comprises dye stuff in a quantity of 1-15% by weight. In the wavelength range between 410 and 680 nm the transmission of the filtering layer comprising said dye is substantially constant and hence spectrally neutral. It has been found that these and other dyes can readily be leached when the filtering layer is in contact with customary cleaning liquids such as ethanol, acetone, diluted acetic acid, ammonium hydroxide, soap and salt water. By incorporating an oxide of Ge, Zr, Al or Ti or a mixture of one or more than one of said metal oxides in the silicon dioxide, a filtering layer is obtained which is better resistant to leaching of the dye. The above metal oxides can be incorporated in the filtering layer on the basis of a mixture of an alkoxysilane and a corresponding alkoxy compounds of said metals, such as tetraethyl orthogermanate Ge(OC₂H₅)₄ (TEOG), tetrabutyl orthozirconate Zr(OC₄H₉)₄ (TBOZ), tetrapropyl orthozirconate Zr(OC₃H₇)₄ (TPOZ), tripropyl orthoaluminate Al(OC₃H₇)₃ (TPOAl) and tetraethyl orthotitanate Ti(OC₂H₅)₄ (TEOTi) in an alcoholic solution. The filtering layer is formed in the hereinafter described manner.

In a favourable embodiment the filtering layer comprises 2-15 mole%, preferably 5-12 mole%, of germanium oxide or zirconium oxide in relation to silicon dioxide. Below 5 mole% the filtering layer is less resistant to cleaning liquids and above 15 mole% no further improvement of the resistance to leaching is obtained and the filtering layer becomes unnecessarily expensive. In addition, above 15 mole% of zirconium oxide, there is a greater risk of gellification of the alcoholic solution after a few hours at room temperature, which would render the solution unsuitable for further processing.

According to the invention, the object of providing a method of manufacturing a filtering layer of silicon dioxide on a display screen of a display device is achieved in that the filtering layer is manufactured by providing, on the display screen, an alcoholic solution of an alkoxysilane compound, an alkoxy compound of at least one metal selected from the group formed by Ge, Zr, Al and Ti, acidified water and a black dye, followed by a treatment at an increased temperature, thereby forming the filtering layer comprising silicon dioxide, an oxide of the metal and the dye.

A suitable alkoxysilane compound for use in the method in accordance with the invention is tetraethyl orthosilicate (TEOS). Other alkoxysilane compounds of the type Si(OR)₄, which are known *per se*, and oligomers thereof can alternatively be used, wherein R represents an alkyl group, preferably a C₁-C₅ alkyl group. Preferably, the alcoholic solution is applied to the display screen by spin coating. After drying and heating to, for example, 160°C for 30 minutes a grey to black, smooth and high-gloss filtering layer is obtained in this manner. To obtain a homogeneous, smooth layer it may be beneficial to add a surface-active substance, for example in quantities of from 0.001 to 5% by weight, to the solution. If desired, the alcoholic solution can be applied by spraying, thereby forming a mat filtering layer having anti-glare properties. For the alcohol, use can be made of ethanol, propanol, butanol, diacetone alcohol or a mixture thereof. Using acidified water the alkoxy groups of Si and the above-mentioned metals are converted into hydroxy groups by hydrolysis. Said hydroxy groups react with each other and with hydroxy groups of the glass surface of the display screen. During drying and heating, polycondensation brings about a satisfactorily adherent oxidic network of silicon dioxide in which oxides of one or more than one of the metals Ge, Zr, Al and Ti and the dye are incorporated. For the alkoxy compounds of the said metals use is made of compounds of the formula:
M(OR)ₙ, where M = Ge, Zr, Al or Ti; R = C₁-C₅ alkyl group and n is the valency of the metal M. The above-mentioned compounds TEOG, TBOZ, TPOZ, TPOAl and TEOTi can be used by way of example. Preferably Orasol Black CN™ (Colour Index: Solvent Black 28) is used as the black dye because it has the above-mentioned favourable properties.

In a favourable embodiment of the method in accordance with the invention, 0.25-1 mole of acetylacetone (2,4-pentanedione) per mole of alkoxy compound of Ge, Zr, Al or Ti is also added to the alcoholic solution. This addition leads to an improved abrasion resistance of the filtering layer formed. The enol form of acetylacetone forms a complex with the metal M, as a result of which the velocity of the hydrolysis reaction and condensation reaction of the relevant M compound is reduced by steric hindrance. This effect promotes the formation of ≡Si-O-M≡ bonds at the expense of the formation of ≡M-O-M≡ bonds, so that covalent incorporation of the metal M into the silica network takes place more readily than the formation of oxide particles by the metal M.

It is assumed that fewer and/or smaller M-oxide particles have a favourable effect on the abrasion resistance. Too much acetylacetone may cause corrosion of the metal vessels and pipelines used, whereas too small a quantity of acetylacetone causes long filtration times of the coating solution due to the formation of many and/or large M-oxide particles. A quantity of 0.5 mole of acetylacetone per mole of M-alkoxy compound is optimal.

If desired, a filtering layer having antistatic properties can be obtained by adding a conductive metal oxide such as tin oxide, indium oxide or antimony oxide, the oxide being suspended in the alcoholic solution of the alkoxy compounds. It is alternatively possible to provide the filtering layer on a separate transparent front plate instead of on the display screen itself.

The invention will be explained in greater detail by means of exemplary embodiments and a drawing, in which the sole

Figure is a partly exploded perspective view of an embodiment of a cathode ray tube in accordance with the invention.

### Exemplary embodiment 1.

### Preparation of germanium alkoxide liquid:

A quantity of 5 grams of tetraethoxygermanate (TEOG) is added to a solution of 2.5 grams of Orasol Black CN™ (supplier Ciba Geigy) in 100 grams of ethanol and 100 grams of 1-butanol. In addition, a solution is prepared which comprises 100 grams of ethanol, 50 grams of tetraethoxy silane (TEOS) and 8 grams of water acidified with 1 N of HCl. After a reaction time of 30 minutes the two solutions are mixed. After 15 minutes a mixture of 8 grams of water acidified with 1 mole/l of HCl, 50 grams of ethanol and 50 grams of diacetone alcohol is added. After a reaction time of 6 hours, the mixture obtained is passed through a PTFE-filter having a pore size of 0.2 µm.

### Preparation of titanium alkoxide liquid:

A quantity of 5 grams of tetraethoxy titanate (TEOTi) is added to a solution of 2.3 grams of Orasol Black CN™ in 100 grams of ethanol and 100 grams of 1-butanol. In addition, a solution is prepared which comprises 100 grams of ethanol, 50 grams of TEOS and 8 grams of water acidified with 1 mole/l of HCl. After a reaction time of 30 minutes, the two solutions are mixed. After 15 minutes, a mixture of 8 grams of water acidified with 1 mole of HCl, 50 grams of ethanol and 50 grams of diacetone alcohol is added. After a reaction time of 6 hours, the mixture obtained is passed through a PTFE filter having a pore size of 0.2 µm.

### Preparation of aluminium alkoxide liquid:

The procedure used for the preparation of titanium alkoxide liquid is repeated, with this difference that 5 grams of tripropoxy aluminate (TPOAl) are used instead of 5 grams of TEOTi.

### Preparation of zirconium alkoxide liquid:

The procedure used for the preparation of titanium alkoxide liquid is repeated, with this difference that 8,5 grams of tetrabutoxy zirconate (TBOZ) are used instead of 5 grams of TEOTi.

The above solutions are spin coated on to clean glass plates of 10 x 10 cm at a speed of 200 r.p.m. for 1 minute. The coated glass plates are heated to 150°C for 20 minutes, thereby forming the cured filtering layers.

All filtering layers thus formed are mirror bright, neutral black and exhibit an average transmission of 70±2% between 420 and 680 nm.

All filtering layers are resistant to washing with weak acid, weak base, ethanol, acetone, water and customary cleaning agents.

By means of a scratch test, in which a diamond needle is moved several times over the filtering layers with a force of 45 grams, it was established that the abrasion resistance of the filtering layers is satisfactory. After said test no damage to the surface could be observed.

The resistance to light of the filtering layers is tested by means of the so-called Xenotest in accordance with DIN-standards 54003 and 54004, using a Heraeus Suntest CPS apparatus. In this test, the filtering layers are exposed to artificial light corresponding to daylight under indoor conditions, in such a manner that a residence time of the filtering layer of 24 hours in this apparatus corresponds to 1 year of indoor conditions as tested according to DIN-wool standards. The results after an exposure corresponding to 4 years of indoor use (DIN-wool scale 6) are listed in Table 1.

**TABLE 1**

| alkoxide | relative increase in transmission after 4 years of indoor use (%) |
|---|---|
| TEOG | 4±2 |
| TPOAI | 10±2 |
| TBOZ | 12±2 |
| TEOTi | 24±2 |
| - | 12±2 |

The results listed in Table 1 show that filtering layers of silicon dioxide with incorporated germanium oxide yield an improved light resistance. Oxides of Al, Zr and Ti have no or negative effect on the light resistance and have a positive effect on the resistance of the filtering layer to cleaning liquids. The best results are obtained with germanium oxide. Filtering layers containing germanium oxide are not subject to discoloration (*i.e*. the relative increase in transmission is less than 10%) after 8 to 10 years of indoor use.

### Exemplary embodiment 2.

In accordance with the method of exemplary embodiment 1, glass plates are provided with filtering layers of silicon dioxide into which zirconium oxide and black dye is incorporated, the zirconium oxide content varying between 5 and 15 mole% in relation to silicon dioxide. To this end, coating liquids having varying TBOZ contents are prepared.
The filtering layer provided must be resistant to cleaning agents and other customarily used liquids. To determine the resistance, drops of ethanol (100%), acetone (100%), acetic acid (50%), ammonium hydroxide (14%), soap solution and salt water are provided on the filtering layer. After the drops have dried the surface of the filtering layer is examined as to whether it has been attacked and/or any dye has been leached. The results regarding leaching are shown in Table 2.

**TABLE 2**

| mol. % Zr | ethanol | acetone | ammonium hydroxide | acetic acid | salt water | soap |
|---|---|---|---|---|---|---|
| 5 | - | - | - | + | + | + |
| 10 | + | + | + | + | + | + |
| 15 | + | + | + | + | + | + |
| In this Table, the symbols have the following meaning: + satisfactory resistance to leaching - poor resistance to leaching. | | | | | | |

The best results were obtained by incorporating 10-15 mol.% of zirconium oxide in relation to silicon dioxide. Higher concentrations lead, after several hours at room temperature, to gellification of the alcoholic solutions.

Ammonium hydroxide slightly attacks the filtering layer, except when the filtering layer contains at least 10 mol. % of germanium oxide.

### Exemplary embodiment 3.

A solution is prepared (solution A) from the following constituents:
- 300 g ethanol
- 170 g 1-butanol
- 75 g TEOS
- 4 g Orasol Black CN™
- 65 g HCl/H₂O solution (1 mole/l)
This mixture is stirred at room temperature for 1 hour.

In addition, a solution is prepared (solution B) from the following constituents:
- 55 g ethanol
- 1.4 g acetylacetone
- 14 g TBOZ

This mixture is also stirred at room temperature for 1 hour. Subsequently, solution B is added to solution A. After stirring for 5 minutes, 80 g of diacetone alcohol is added. The mixture obtained is stirred for 10 minutes and then passed through a PTFE-filter having a pore size of 0,2 µm.

In the same manner as described in exemplary embodiment 1, the solution obtained is used to coat glass plates.

The layer obtained has an excellent abrasion resistance which is determined by rubbing the filtering layer twenty times with a rubber eraser (Lion special No. 50) with a force of 10 N. After said test, the filtering layer was examined under the microscope (magnetification 100 x) and no scratches could be observed.

If, under equal conditions, no acetylacetone is added to the coating solution a few scratches having a width of 2 µm are visible.

The addition of acetylacetone to the coating solution leads to a coating having a better abrasion resistance, while the other properties are not adversely affected.

### Exemplary embodiment 4.

The Figure diagrammatically shows an exploded perspective view of a cathode ray tube which is known *per se* and which has a glass envelope 31 comprising a display screen 32, a cone 33 and a neck 34. In the neck there is provided an electron gun 35 for generating an electron beam 36. This electron beam 36 is focused on to a target spot 38 on a phosphor layer 37 on the inner surface of the display screen 32. The electron beam 36 is deflected across the display screen 32 in two mutually perpendicular directions x-y by means of the deflection coil system 39. The outer surface of the display screen 32 is provided with a filtering layer 40 which is manufactured as described in any of the above exemplary embodiments.

The invention enables spectrally neutral filtering layers to be manufactured and provided on a display screen of a display device in a simple manner. Said filtering layers may be mirror bright, are resistant to light and to customary cleaning liquids. Curing the filtering layer at 160°C, a temperature to which display tubes are resistant, results in scratch-resistant layers.

## Claims

1. A display device comprising a display screen which is provided with a filtering layer comprising silicon dioxide, a black dye and a metal oxide, characterized in that the metal of the oxide is selected from the group formed by Ge, Zr, Al and Ti.

2. A display device as claimed in Claim 1, characterized in that the black dye is a mono-azo chromium complex with a Colour Index: Solvent Black 28.

3. A display device as claimed in Claim 1, characterized in that the filtering layer contains 2-15 mol.% of germanium oxide in relation to silicon dioxide.

4. A display device as claimed in Claim 1, characterized in that the filtering layer contains 2-15 mol.% of zirconium oxide in relation to silicon dioxide.

5. A method of manufacturing a filtering layer of silicon dioxide on a display screen of a display device, wherein the filtering layer is manufactured by providing, on the display screen, an alcoholic solution of an alkoxysilane compound, an alkoxy compound of at least one metal selected from the group formed by Ge, Zr, Al and Ti, acidified water and a black dye, followed by a treatment at an increased temperature, thereby forming the filtering layer comprising silicon dioxide, an oxide of the metal and the dye.

6. A method as claimed in Claim 5, characterized in that a mono-azo chromium complex with a Colour Index: Solvent Black 28 is used as the black dye.

7. A method as claimed in Claim 5, characterized in that a tetraalkoxy zirconate or tetraalkoxy germanate is used as the alkoxy compound.

8. A method as claimed in Claim 5, characterized in that 0.25-1 mole of acetylacetone per mole of alkoxy compound of Ge, Zr, Al or Ti is also added to the alcoholic solution.

## Patentansprüche

1. Bildwiedergabeanordnung mit einem Bildschirm mit einer Filterschicht mit Siliziumdioxid, einem schwarzen Farbstoff und mit einem Metalloxid, dadurch gekennzeichnet, daß das Metall des Oxids aus der Gruppe gewählt worden ist, die durch Ge, Zr, Al und Ti gebildet wird.

2. Bildwiedergabeanordnung nach Anspruch 1, dadurch gekennzeichnet, daß der schwarze Farbstoff ein Mono-azo-chromkomplex mit einem Farbindex: Solvent Black 28 ist.

3. Bildwiedergabeanordnung nach Anspruch 1, dadurch gekennzeichnet, daß die Filterschicht 2 - 15 Mol% Germaniumoxid gegenüber Siliziumdioxid aufweist.

4. Bildwiedergabeanordnung nach Anspruch 1, dadurch gekennzeichnet, daß die Filterschicht 2 - 15 Mol% Zirkonoxid gegenüber Siliziumdioxid aufweist.

5. Verfahren zum Anbringen einer Filterschicht aus Siliziumdioxid auf einem Wiedergabeschirm einer Bildwiedergabeanordnung, wobei die Filterschicht dadurch hergestellt wird, daß am Wiedergabeschirm eine Alkohollösung aus einer Alkoxysilanverbindung, einer Alkoxyverbindung von wenigstens einem Metall, selektiert aus der Gruppe, die durch Ge, Zr, Al und Ti gebildet wird, aus angesäuertem Wasser und aus einem schwarzen Farbstoff vorgesehen wird, wonach eine Behandlung bei erhöhter Temperatur folgt, wodurch die Filterschicht mit Siliziumdioxid, mit einem Oxid des Metalls und mit dem Farbstoff gebildet wird.

6. Verfahren nach Anspruch 5, dadurch gekennzeichnet, daß ein Mono-azo-chromkomplex mit einem Farbindex: Solvent Black 28 als schwarzer Farbstoff verwendet wird.

7. Verfahren nach Anspruch 5, dadurch gekennzeichnet, daß als Alkoxyverbindung ein Tetraalkoxyzirkonat oder ein Tetraalkoxygermanat verwendet wird.

8. Verfahren nach Anspruch 5, dadurch gekennzeichnet, daß 0,25 - 1 Mol Azetylazeton je Mol Alkoxyverbindung von Ge, Zr, Al oder Ti zu der Alkohollösung hinzugefügt wird.

## Revendications

1. Dispositif d'affichage comportant un écran d'affichage qui est muni d'une couche filtrante comportant du bioxyde de silicium, une teinture noire et un oxyde métallique, caractérisé en ce que le métal de l'oxyde est choisi du groupe étant formé par Ge, Zr, Al et Ti.

2. Dispositif d'affichage selon la revendication 1, caractérisé en ce que la teinture noire est un complexe de chromium mono-azoïque présentant un indice de couleur: Solvent Black 28.

3. Dispositif d'affichage selon la revendication 1, caractérisé en ce que la couche filtrante contient 2 à 15% en moles d'oxyde de germanium par rapport au bioxyde de silicium.

4. Dispositif d'affichage selon la revendication 1, caractérisé en ce que la couche filtrante contient 2 à 15% en moles d'oxyde de zirconium par rapport au bioxyde de silicium.

5. Procédé pour fabriquer une couche filtrante en bioxyde de silicium sur un écran d'affichage d'un dispositif d'affichage où la couche filtrante est fabriquée par l'application, sur l'écran d'affichage, d'une solution alcoolique constituée d'un composé d'alcoxysilane, d'un composé d'alcoxy égal à au moins un métal choisi du groupe étant formé par Ge, Zr, Al et Ti, par de l'eau acidifiée et par une teinture noire, ce qui est suivi d'un traitement à une température plus élevée du fait qu'il est constitué de ce fait la couche filtrante comportant du bioxyde de silicium, un oxyde du métal et la teinture.

6. Procédé selon la revendication 5, caractérisé en ce qu'un complexe de chromium mono-azoïque présentant un indice de couleur: Solvent Black 28 est utilisé comme la teinture noire.

7. Procédé selon la revendication 5, caractérisé en ce qu'un zirconate de tétra-alcoxy ou un germanate de tétra-alcoxy est utilisé comme le composé d'alcoxy.

8. Procédé selon la revendication 5, caractérisé en ce qu'une quantité comprise entre 0,25 et 1 mole d'acétyle-acétone par mole de composé d'alcoxy de Ge, de Zr, d'Al ou de Ti est également ajoutée à la solution alcoolique.
